

1

3,082,171

## MAGNETIC LITHOGRAPHIC INK

Clarence J. Shoemaker, Elmhurst, and Tadeusz Hoffmann, Chicago, Ill., assignors to A. B. Dick Company, Niles, Ill., a corporation of Illinois  
 No Drawing. Continuation of application Oct. 14, 1958, Ser. No. 767,093. This application Aug. 23, 1960, Ser. No. 51,291

2 Claims. (Cl. 252—62.5)

This invention relates to magnetic ink for use in lithographic duplicating machines to produce copy capable of being read with the magnetic reading head in automatic, high speed, scanning devices.

This is a continuation of my copending application Serial Number 767,093, now abandoned, entitled Magnetic Lithographic Ink, filed October 14, 1958.

It relates more particularly to a lithographic duplicating ink embodying characteristics essential for use with magnetic read-out devices and a component or better wet-out of the paper to produce a full image such as would be desirable for successful operation in magnetic read-out.

It is an object of this invention to produce a magnetic ink having lithographic properties for use in lithographic duplicating machines to produce magnetic printing, and it is a related object to produce a lithographic ink of the type described containing a magnetic component in the form of a magnetic iron oxide; which produces easily readable and well defined copy; which produces a full and complete image; which does not feed back into the fountain solution of the lithographic duplicating machine thereby to keep the fountain free of contaminating magnetic particles; which produces copy having sufficient magnetic strength for efficient and proper read-out, and which is capable of producing a large number of copies of good quality.

In accordance with the practice of this invention, a magnetic ink for lithographic duplication is formulated of the combination of the following materials present in amounts as hereinafter set forth.

## EXAMPLE 1

## Magnetic Ink Composition (Broad)

Percent by weight

|                                 |       |
|---------------------------------|-------|
| Lithographic vehicle or varnish | 20-60 |
| Magnetic iron oxide             | 25-70 |
| Toners or tinctorial agents     | 1-20  |
| Lecithin                        | 1-5   |

Lithographic ink varnishes are well known to the trade. They usually comprise a base capable of fluid flow. The base may be a bodied oil, such as linseed oil, or a hydrocarbon, or an oil from the synthetic resinous materials such as alkyd resin or a phenol formaldehyde resin. The following are classes of varnishes which can be used:

Linseed modified phenol formaldehyde varnish

Bodied linseed oil varnish

Maleic-alkyd varnish

Pentaerythritol alkyd varnish

Hydrocarbon varnish

It is preferred to make use of a lithographic varnish giving a high degree of water repellency to the copy. A suitable varnish is marketed by General Printing Ink Company under the designation No. 01269.

As to the magnetic iron oxide, use can be made of

2

special grades of iron oxide identified as acicular iron oxide which can be prepared from commercial grades of iron oxide by known reduction and oxidation techniques. A suitable material is marketed by C. K. Williams Company of Easton, Pennsylvania, under the trade name IRN100.

The toner comprises a tinctorial agent to impart a desired shade and readability to the copy. Use can be made of such conventional toners as carbon black, lamp black, alkali blue, iron blue, and other dyestuffs and pigments. They may be incorporated as a dry pigment or as a dispersion in varnish oils for introduction into the composition.

The surface active agent functions also as a wetting agent for the pigment, and for wet-out of the surface upon which the magnetic ink is deposited in printing to produce a full and complete image. For this purpose, best use can be made of a lecithin. A suitable material (soy bean lecithin) is marketed by American Lecithin Company, Long Island City, New York, under the trade name "Alcolec 410N."

The following are specific examples of magnetic lithographic inks prepared in accordance with the practice of this invention:

## EXAMPLE 2

|                     | Percent |
|---------------------|---------|
| P. E. alkyd varnish | 37      |
| Linseed oil         | 10      |
| Lecithin            | 1       |
| Carbon black        | 1       |
| Iron blue           | 1       |
| Iron oxide          | 50      |
|                     | 100     |

## EXAMPLE 3

|                                   | Percent |
|-----------------------------------|---------|
| Linseed modified phenolic varnish | 27      |
| Linseed oil                       | 15      |
| Iron oxide—IRN100                 | 56      |
| Lecithin                          | 1       |
| Alkali blue                       | 1       |
|                                   | 100     |

45 It will be understood that the amounts of the components may be varied within the range described to provide the desired viscosity characteristics which can best be determined by trial and error.

For example, in a preferred range, the varnish made up of bodied oil or a resin or oil modified resin, alone or in combination with an oil, such as linseed oil, may be employed in an amount within the range of 20-45% by weight; the magnetic iron oxide may be employed in an amount within the range of 45-60% by weight; the surface active agent, such as lecithin, may be employed in an amount within the range of 1-5% by weight, and the tinctorial agent, such as carbon black, iron blue and the like, alone or in combination, may be employed in an amount within the range of 1-5% by weight.

60 The materials may be incorporated in any order but it is best to mix all of the ingredients and then to grind the material in conventional machines for the preparation of an ink.

It will be understood that changes may be made in the details of the formulation and composition without depart-

ing from the spirit of the invention, especially as defined in the following claims.

We claim:

1. A magnetic, lithographic ink consisting essentially of the combination of 20-60% by weight lithographic varnish, 25-70% by weight magnetic iron oxide, 1-20% by weight tinctorial agent, and 1-5% by weight lecithin.

2. A magnetic, lithographic ink consisting essentially of the combination of 20-45% by weight lithographic varnish, 45-60% by weight magnetic iron oxide, 1-5% by weight tinctorial agent, and 1-5% by weight lecithin.

References Cited in the file of this patent

UNITED STATES PATENTS

5 2,649,381 Hempel et al. \_\_\_\_\_ Aug. 18, 1953  
5 2,688,649 Bjorksten \_\_\_\_\_ Sept. 7, 1954

OTHER REFERENCES

Wolfe: Printing and Litho Inks, 4th ed., Macnair Dor-  
land Co., New York, N.Y., 1949, pp. 43-49, 103-105,  
161-162, 176-183, 187, 205, 232, 270-276.